

1

2,864,675

## ADDITIVE FOR GASOLINE AND DIESEL FUELS

James W. Jean, Altadena, Calif., assignor, by direct and mesne assignments, of fifty-one percent to A. R. Chandler, thirty-two percent to John N. Adams, and seventeen percent to Stanley Turner

No Drawing. Application October 24, 1955  
Serial No. 542,508

12 Claims. (Cl. 44—50)

This invention relates to an addition agent for fuels for internal combustion engines of both the spark ignition type and the diesel type, and more particularly to hydrocarbon fuels boiling in the gasoline boiling range and to diesel fuels.

This application is a continuation in part of my copending application, Serial No. 314,569, filed October 13, 1952, for improvements in Additive for Both Gasoline and Diesel Fuels, and now abandoned.

The usual additive for fuel for internal combustion engines is not adaptable for both gasoline and diesel fuels. For example, an additive for gasoline to improve its anti-knock characteristics by causing a more progressive travel of the ignition or so-called "flame front" throughout the mass of fuel within the engine cylinder, and therefore reducing the tendency toward explosion simultaneously through the mass of the fuel, would not be useful in non-spark ignition engines, such as diesel engines, where ignition and explosion of the fuel are brought about by the heat of compression of the air. Instead, such an anti-knock agent for gasoline would have an effect just the reverse of what is desired in diesel fuels.

It is an object of this invention to produce an additive for motor fuels which gives substantially the same improvement in the operation of the engine, irrespective of whether the engine is of the gasoline type or the diesel type. Among the advantages of my additive with both types of engine are ease of starting, suppression of carbon deposition, elimination of gum formation, marked smoothness in operation and increased power output.

Diesel fuels are often not so highly refined as gasoline fuel and therefore are frequently attended by foul odor, due in part at least, to the presence of sulfur compounds. It is another object of my invention to produce an additive for diesel fuels which eliminate foul odor both in light and in the heavier diesel fuels.

According to the present invention, my additive is obtained through the action that takes place between urea, an alkali metal hydroxide, alcohols and ketones in the presence of a suitable solvent.

As an example of a specific embodiment of my invention, the following is given for the preparation of approximately a one-gallon batch of the additive: To 16 ounces (1 lb.) dry commercial urea, such as that manufactured and sold as containing 44% of nitrogen, there are added four ounces of dry sodium hydroxide. There is then added a liquid mixture consisting of 1300 cc. of isopropyl alcohol, 1300 cc. of methyl ethyl ketone and 1300 cc. of a petroleum distillate fraction such as that sold under the trade name "Amsco Solv A-80," said petroleum distillate fraction being commonly used as a solvent for paint thinners because of its high content of aromatic hydrocarbons, this particular distillate fraction having an A. P. I. gravity of 40.5, and an initial boiling point, by the A. S. T. M. distillation method, of 213° F., an end point of 242° F. and an aromatic hydrocarbon content, as shown by its aniline point, of

2

77%, most of which aromatic content being reported by said company's laboratory as toluene. The mass is then stirred and allowed to stand at room temperature until it has attained a color throughout its entire mass ranging from a medium to dark red, depending upon time of standing and temperature of the room—usually from 24 to 48 hours. It will be noted that no heat is applied and that no water is present except such traces of moisture as may exist in the ingredients employed.

As the reaction proceeds color changes take place, a pale cream color rising at the beginning from the urea and sodium hydroxide up into the liquid mass and the liquid mass finally becoming a clear dark red solution with some reddish flocculent material suspended in it. The red solution with its aforesaid flocculent suspended material is drained off from excess urea and sodium hydroxide that remain in the bottom of the vessel. The red solution is then filtered to remove the reddish flocculent material, which latter is a red amorphous powder. The clear dark red solution is a very stable material and constitutes the additive obtained from the materials of this example which I employ for both gasoline and diesel fuels. It is substantially completely soluble in all grades of petroleum motor fuels, from gasoline on through the various grades of diesel fuels.

Just what chemical reaction takes place in the formation of the red liquid which comprises this additive has not been definitely determined. No gas bubbles arise during the process, indicating that no free ammonia or other gaseous substance is formed. Both the product and the reaction involved have definite characteristics. When prepared in the aforesaid manner substantially all of the clear red liquid is oil soluble. When water is added to this red liquid no clear solution is formed. Instead, it becomes cloudy, and upon standing the water settles to the bottom. If before filtering out the solids as above explained a relatively large volume of water is added and shaken, the solids will dissolve and a two-phase system formed, an oily layer forming at the top. Upon removing this top layer and letting the remainder stand at room temperature some entrained water will settle to the bottom, leaving the clear red liquid. It would thus appear that the red liquid is substantially insoluble in water. In view of the fact that the urea, the sodium hydroxide, the isopropyl alcohol and the methyl ethyl ketone are all water soluble this non-solubility in water of the resulting red liquid is an unexpected property. When the red liquid is evaporated to dryness, white, long, flat crystals are left which have a distinct pattern. A mass spectrometer examination of the red liquid made in accordance with the above example showed a methyl ethyl ketone content of only 3.5% (from an original 33½%), an increase in the isopropyl alcohol content to 40.8% (from an original 33½%) and a toluene content of only 7% whereas the 33½% of Amsco Solvent A ingredient originally contained around 77% of toluene, and with unknown compounds representing 48% of the sample subjected to the mass spectrometer examination. It is believed that urea adducts are not formed. For one thing such adducts are not understood to be formed when the material of the aforesaid example are employed with urea. Moreover, the presence of sodium hydroxide is not understood to be conducive to the formation of urea adducts; also, the aforesaid non-solubility in water is contrary to the behavior of urea adducts.

The presence of the solvent along with the four reactants appears to exercise an important function in the formation and characteristics of the red liquid. As stated above the red liquid prepared in accordance with the above preferred method is soluble in its entirety in gasoline and all grades of diesel fuel. When, however, the

solvent is not present along with the four ingredients a reddish liquid is formed, but it is not completely soluble in the gasoline or diesel fuels. On the other hand from 75 to 80% of it is water soluble. This suggests that the solvent does not enter the reaction but plays some part in taking up (dissolving) an intermediate reaction product during the progress of the reactions, which intermediate product, in the absence of the solvent, would have ended as water-soluble instead of oil-soluble. In the complete absence of a solvent the relatively small amount of the red liquid formed which is soluble in the motor fuels may be separated from the water-soluble product and used as the additive for motor fuels. Again, when the solvent is not present during the reaction that takes place between the urea, sodium hydroxide, alcohol and ketone such red liquid as is formed is accompanied by the formation of crystals along the sides of the vessel which are of a pale yellow color. These crystals are water-soluble, forming a lemon colored solution but are not soluble in gasoline. They do not form when the solvent is present. Instead, the aforesaid flocculent material forms and is suspended in the red liquid and upon separation by filtering becomes an amorphous red powder. This amorphous red material is water soluble but is not soluble in gasoline or other petroleum products.

If either the alcohol or the ketone is omitted the results will be different from those which are obtained between the urea, sodium hydroxide, alcohol and ketone for the aforesaid conditions, i. e. at room temperature (no heat added) and with no water added. This is true whether or not the solvent is also present. If the ketone is omitted (the alcohol being present) a reaction proceeds which is slower than when the ketone is also present and a yellowish (instead of red) colored liquid results which is mostly water-soluble, less than half of it being soluble in gasoline. When the alcohol is omitted (the ketone being present) the action produces a red colored liquid but again it is mostly water-soluble, less than half of it being soluble in gasoline. With the solvent being also present during the process less of the liquid product formed is water-soluble and more of it is soluble in gasoline, but it is not entirely soluble in gasoline as in the case where both the ketone and the alcohol are present. What reaction takes place between the urea, sodium hydroxide and alcohol (ketone not present) with or without the presence of a solvent, is not known.

Whereas in the formation of my additive no water is present or is added as a separate material, it is possible that small amounts of water present in the materials used may influence or start the reaction. The alcohols which I have employed have been of the 98% grade (2% water). Also, to the extent that true aldol condensation may take place with respect to the ketone or other ingredients some water would be liberated that might perhaps influence the reactions.

Other alcohols may be employed than that of the aforesaid example. While I have obtained excellent results with isopropyl alcohol and prefer to employ it in the production of the additive, I have experienced satisfactory results when there was substituted for the isopropyl alcohol the following alcohols: normal propyl, normal butyl, isobutyl, secondary butyl, tertiary butyl and normal, secondary and tertiary amyl—in other words, any of the alcohols containing from 3 to 5 carbon atoms. While ethyl alcohol may also be employed, it tends to pick up water and is difficult to separate.

Likewise I am not limited to the methyl ethyl ketone of the preferred embodiment of my invention, and have substituted other ketones therefor with satisfactory results. For example, in using acetone cyclohexone or methyl isobutyl ketone, I have obtained a clear liquid of somewhat darker red color than with methyl ethyl ketone but one which gave satisfactory performance as an additive for both gasoline and diesel fuels. Aldehydes may be substituted for the ketones. For example, acetalde-

hyde with isopropyl alcohol gave a product which, although slightly different in appearance from that produced when methyl ethyl ketone was used, was the characteristic red color and worked satisfactorily.

The solvent that may be employed along with the alcohol and ketone to form the three-component liquid mixture to be contacted with the urea and alkali metal hydroxide is susceptible of wide variation. Solvents of different aromatic hydrocarbon content than that of the paint thinner solvent whose gravity and boiling points are specified in the aforesaid example, have been employed with satisfactory results. Petroleum distillate fractions having an aromatic hydrocarbon content as shown by their aniline point, as low as 50%, may be employed as well as those with an aromatic hydrocarbon content of 98%. Petroleum distillate fractions with an aromatic hydrocarbon content falling within this suitable range are those with an A. P. I. gravity range of about 27.5 to 42.5 at 60/60° F. and with an initial boiling point (A. S. T. M. method) ranging from about 210° F. to 355° F., and an end point ranging from about 240° F. to 415° F. I have also had excellent results using straight toluene (commercial grade), as well as benzene. Examples of still other suitable solvents are the xylenes (ortho, meta and para) and the other homologs of benzene such as ethylbenzene, propylbenzene, isopropylbenzene (cumene), pseudocumene and mesitylene. I have also prepared several batches of the additive using kerosene as the solvent; also gasoline, both leaded and unleaded. The same deep red color was obtained in the clear liquid and the engines with which it was used ran with substantially the same smoothness as when the solvent employed was of the aforesaid aromatic hydrocarbon type. While there may be a possibility of some urea adduct formation with kerosene and gasoline as the solvents it is believed, as explained hereinabove, that such is not formed in any substantial amount.

Considerable latitude may be exercised in the relative amounts of the alcohols and ketones or aldehydes employed as well as the amount of solvent used in conjunction therewith to constitute the three-component liquid mixture to be contacted with the urea and alkali-metal hydroxide. I have employed a mixture of the three liquids wherein the alcohol and the ketone or aldehyde were each as low as 12½%, the solvent used therewith comprising the remaining 75%. With such a mixture the resulting red liquid was of a less dense red color than that obtained with higher contents of alcohol and ketone, but upon distilling out the solvent the red color deepened. With 50% solvent, 25% alcohol and 25% ketone or aldehyde, the resulting red liquid is substantially all soluble in gasoline and diesel motor fuels and the effect upon engine performance is substantially the same as when the solvent, alcohol and ketone are in equal volumes, i. e. 33½% each, in the liquid mixture contacted with the urea and alkali-metal hydroxide. The amount of solvent employed should preferably be such as to give complete solubility of the red liquid formed in gasoline and diesel fuels. Generally it should not fall far below about 25% of the entire liquid mixture of solvent, alcohol and ketone or aldehyde employed for desirable solubility of the red liquid in the motor fuels. With such low content of solvent in the mixture the alcohol and ketone content may each be in the neighborhood of 37½%, or they may vary therefrom with respect to each other. My experiments indicate that with an amount of either alcohol or ketone less than 10% of the three-component liquid mixture an insufficient amount of desired reaction product would be produced. In this connection it has been observed that when the amount of ketone exceeds the amount of alcohol the clear red liquid formed is of a deeper red color. I prefer to use a liquid mixture in which the three components are in approximately equal volumes, i. e. 33½% for each.

As regards the alkali metal hydroxides, I have found

that potassium hydroxide may be used in lieu of the sodium hydroxide hereinabove referred to. With lithium hydroxide I have experienced somewhat poor solubility in the mixture as well as poor engine performance. Ammonium hydroxide would not be satisfactory for the reason that the water present would change the conditions making it necessary to apply heat to obtain reaction. Heat would also be necessary if an alkali metal carbonate were used and heat would bring about decomposition or otherwise interfere with the process.

With regard to the amount of urea and alkali metal hydroxide that may be used in proportion to the amount of liquid mixture of alcohol, ketone and solvent employed, in the example first hereinabove given, which as stated, is for the production of one gallon of the clear red liquid, the amounts of urea and sodium hydroxide stated are in excess of that which enters into the reaction. If smaller quantities of urea are employed the clear red liquid formed is of somewhat lighter color. On the other hand when a larger amount of urea is used no deepening of the red color takes place, indicating that the reaction will go only so far regardless of higher proportions of urea present. My experiments indicate that for the liquid mixture in an amount as stated for the aforesaid example an upper limit of 20 oz. of urea would be sufficient to attain a maximum amount of reaction. For satisfactory practical results the amount of urea, for the aforesaid amount of liquid mixture should not be less than about 6 ounces. In general the amount of urea may range from a maximum of about 15% of the weight of the entire liquid mixture (solvent plus alcohol plus ketone) to a minimum of about 5% of the weight of said liquid mixture.

While the alkali metal hydroxide appears to act catalytically, the amount employed does have an effect upon the rate of the reaction, it being faster with larger amounts. No harmful effects on the product formed result from the use of an excess of the alkali. If too little is used, the reaction is slowed. For satisfactory practical purposes, for the amount of liquid mixture added as per the example hereinabove given, the amount should not drop below about 1 ounce, whereas around 10 ounces is an upper limit beyond which there would be no need to go. Thus the alkali metal hydroxide may range from about one-half to one-sixth of the amount of urea.

With respect to the rate of use of the material as an additive for internal combustion engine fuel: When used in gasoline excellent results are obtained when it is employed at the rate of 1 cc. of the aforesaid red liquid in 10 gallons of gasoline. The increase in power output is so marked that I have found it advisable not to use it in amounts greater than 3 cc. in 10 gallons of gasoline, which is approximately 1 volume to 38,000 volumes of gasoline. Very satisfactory results have been obtained when it is employed at the rate of 0.5 cc. per 10 gallons of gasoline, i. e. at 1 volume to 76,000 volumes of gasoline.

When used in diesel fuels, a satisfactory rate ranges from 6 cc. to 12 cc. per 10 gallons of fuel depending on the type of fuel employed. Lighter diesel fuels will require less whereas with the heavier fuels greater dosages can be used for best results. Diesel fuels in general being heavier than gasoline, are harder to burn and give rise to more carbon formation, hence more of the additive is used than with gasoline. The additive is particularly beneficial in the starting of cold diesel engines, some diesel engines being extremely hard to start when cold.

The use of the clear red liquid prepared in accordance with the foregoing procedure from the stated materials gives an additive that is highly beneficial when used with either gasoline or hydrocarbon diesel fuels, giving marked smoothness of operation and increased power output in gasoline engines and in diesel engines. It is particularly pronounced in preventing gum formation and in sup-

pressing carbon deposition in both types of engines. Additionally, it acts as a stabilizer against chlorine and bromine compounds that form from tetra ethyl lead contained in some gasoline. Being alkaline it inhibits or counteracts acid conditions resulting from sulfur compounds in fuels, particularly in less refined diesel fuels. It is also particularly beneficial in the starting of cold diesel engines. This has been effectively demonstrated in the operation over a period of twenty-two months of

- 10 two trucks each powered by a 150 H. P. Cumming engine. The starting of the engine of these trucks was improved remarkably when the diesel fuel contained the additive made in accordance with this invention. The trucks operaeted more smoothly and seemed to have considerably 15 more power on hills. At the conclusion of the 22-month operation with this additive, the engines were found to be clean. The fuel used in these diesel engines during this test period was a #2 furnace oil of about 32 gravity purchased from a major oil company.
- 20 The diesel engine fuel suitable for use with my additive may be described broadly as petroleum distillates boiling in the range of from about 350° F. to about 750° F. Such distillates are ordinarily characterized by an A. P. I. gravity of at least 20°, and usually at least 25°, the base stocks being either straight-run distillates or cracked distillates.

With respect to the fuel for spark ignition engines suitable for use with my additive, I have herein used the terms gasoline and hydrocarbon fuels boiling in the gasoline boiling range. These terms are intended to be used interchangeably and where the term gasoline is used both are understood to be embraced. These fuels have an A. S. T. M. distillation with an initial boiling point of about 100° F., and a final boiling point of about 400° F. 30 and they may embrace for example straight run or cracked petroleum distillates, catalytically re-cracked gasoline distillate to convert olefinic constituents of the distillate, an alkylate (e. g. isoparaffin-olefin alkylate), an aromatic fuel (e. g. cumene, toluene, m- and p-xylene, etc.), hydro- 35 genated polymers (e. g. polymers of butene which, upon hydrogenation, have characteristics of iso-octane, etc.), iso- 40 pentane or butane, or a blend of two or more of such, or other, types of fuels.

Having thus described my invention, it will be understood that the invention embraces such variations and modifications as come within the spirit and scope thereof.

- I claim:
1. The method of making an additive suitable for a spark ignition engine hydrocarbon fuel boiling in the 50 gasoline boiling range and for a diesel engine fuel, which comprises admixing substantially dry urea and a dry alkali metal hydroxide selected from the group consisting of sodium hydroxide and potassium hydroxide with a liquid mixture consisting essentially of an alcohol containing from three to five carbon atoms, a ketone containing up to six carbon atoms and a solvent selected from the group consisting of a petroleum distillate fraction having an A. S. T. M. distillation with an initial boiling point within the range of about 210° F. to 355° 55 F., an end point within the range of about 240° F. to 415° F., an A. P. I. gravity within the range of about 27.5 to 42.5 at 60/60° F. and an aromatic hydrocarbon content above about 50%, benzene, a homolog of benzene, gasoline and kerosene, the amount of said urea being within the range of from about 5% to 15% of the weight of said liquid mixture, the amount of said alkali metal hydroxide being within the range of from about 60 65 one-sixth to one-half of the weight of said urea, the said solvent component of said liquid mixture comprising from about 25% to about 75% by volume of said liquid mixture, and the alcohol and ketone components comprising each in excess of about 10% by volume of said liquid mixture, allowing the admixture to stand at ordinary room temperature until a clear reddish colored liquid 70 is formed, and separating the resultant clear red liquid 75

from any newly formed solid material and residual material.

2. The method in accordance with claim 1 wherein the alkali metal hydroxide is sodium hydroxide.

3. The method in accordance with claim 1 wherein the said solvent component of said liquid mixture is essentially toluene.

4. The method in accordance with claim 1 wherein the said solvent component of said liquid mixture is essentially a petroleum distillate fraction having an A. S. T. M. distillation with an initial boiling point within the range of about 210° F. to 355° F., an end point within the range of about 240° F. to 415° F., an A. P. I. gravity within the range of about 27.5 to 42.5 at 60/60° F. and an aromatic hydrocarbon content above about 50%.

5. An addition agent for spark ignition engine hydrocarbon fuel boiling within the gasoline boiling range and for diesel fuel, said addition agent having been prepared by admixing substantially dry urea and a dry alkali metal hydroxide selected from the group consisting of sodium hydroxide and potassium hydroxide with a liquid mixture consisting essentially of an alcohol containing from three to five carbon atoms, a ketone containing up to six carbon atoms and a solvent selected from the group consisting of a petroleum distillate fraction having an A. S. T. M. distillation with an initial boiling point within the range of about 210° F. to 355° F., an end point within the range of about 240° F. to 415° F., an A. P. I. gravity within the range of about 27.5 to 42.5 at 60/60° F. and an aromatic hydrocarbon content above about 50%, benzene, a homolog of benzene, gasoline and kerosene, the amount of said urea being within the range of from about 5% to 15% of the weight of said liquid mixture, the amount of said alkali metal hydroxide being within the range of from about one-sixth to one-half of the weight of said urea, the said solvent component of said liquid mixture comprising from about 25% to about 75% by volume of said liquid mixture, and the alcohol and ketone components comprising each in excess of about 10% by volume of said liquid mixture, allowing the admixture to stand at ordinary room temperature until a clear reddish colored liquid is formed, separating the resultant clear red liquid from any newly formed solid material and residual material.

6. An addition agent in accordance with claim 5 wherein the solvent, the alcohol and the ketone each constitutes about 33½% by volume of the said liquid mixture employed in the preparation of said addition agent.

7. An addition agent in accordance with claim 5 wherein the solvent constitutes about 75% by volume of the said liquid mixture employed in the preparation of said addition agent and the alcohol and ketone components of said liquid mixture are in about equal volumes.

8. An addition agent in accordance with claim 5 wherein the solvent constitutes about 50% by volume of the said liquid mixture employed in the preparation of said addition agent and the alcohol and ketone components are each in excess of about 10% by volume of said liquid mixture.

9. An addition agent in accordance with claim 5 wherein the solvent constitutes about 25% by volume of the said liquid mixture employed in the preparation of said addition agent and the alcohol and ketone components are each in excess of about 10% by volume of said liquid mixture.

10. An addition agent for spark ignition engine hydrocarbon fuel boiling within the gasoline boiling range and for diesel fuel, said addition agent having been prepared by admixing substantially dry urea and a dry alkali metal hydroxide selected from the group consisting of sodium hydroxide and potassium hydroxide with a liquid mixture consisting essentially of an alcohol containing from three to five carbon atoms and a ketone containing up to six carbon atoms, the amount of said urea being within the range of from about 5% to 15% of the weight of said liquid mixture, the amount of said alkali metal hydroxide being within the range of from about one-sixth to one-half of the weight of said urea, the said alcohol and said ketone each constituting in excess of about 10% by volume of said liquid mixture, allowing the admixture to stand at ordinary room temperature until a clear reddish colored liquid is formed, separating the resultant clear red liquid from any newly formed solid material and residual material, and freeing said resultant clear red liquid of its water soluble portion.

11. An addition agent in accordance with claim 10 wherein the alcohol and ketone each constitutes about one-half by volume of said liquid mixture.

12. An addition agent for spark ignition engine hydrocarbon fuel boiling within the gasoline boiling range and for diesel fuel, said addition agent having been prepared by admixing substantially dry urea and a dry alkali metal hydroxide selected from the group consisting of sodium hydroxide and potassium hydroxide with a liquid mixture consisting essentially of an alcohol containing up to five carbon atoms, a ketone containing up to six carbon atoms and a solvent selected from the group consisting of a petroleum distillate fraction having an A.S.T.M. distillation with an initial boiling point within the range of about 210° F. to 355° F., an end point within the range of about 240° F. to 415° F., and A. P. I. gravity within the range of about 27.5 to 42.5 at 60/60° F. and an aromatic hydrocarbon content above about 50%, benzene, a homolog of benzene, gasoline and kerosene, the amount of said urea being within the range of from about 5% to 15% of the weight of said liquid mixture, the amount of said alkali metal hydroxide being within the range of from about one-sixth to one-half of the weight of said urea, the said solvent component of said liquid mixture comprising from about 25% to about 75% by volume of said liquid mixture, and the alcohol and ketone components comprising each in excess of about 10% by volume of said liquid mixture, allowing the admixture to stand at ordinary room temperature until a clear reddish colored liquid is formed, and separating the resultant clear red liquid from any newly formed solid material and residual material.

References Cited in the file of this patent

UNITED STATES PATENTS

|    |           |               |       |                |
|----|-----------|---------------|-------|----------------|
| 55 | 974,749   | Caulfield     | ----- | Nov. 1, 1910   |
|    | 1,469,053 | Schreiber     | ----- | Sept. 25, 1923 |
|    | 1,684,686 | Records       | ----- | Sept. 18, 1928 |
|    | 2,002,645 | Rather et al. | ----- | May 28, 1935   |
| 60 | 2,447,621 | Smidt         | ----- | Aug. 24, 1948  |
|    | 2,529,784 | Olin et al.   | ----- | Nov. 14, 1950  |

FOREIGN PATENTS

|    |         |               |       |               |
|----|---------|---------------|-------|---------------|
| 65 | 562,091 | Great Britain | ----- | June 19, 1944 |
|----|---------|---------------|-------|---------------|